

C. F. GEISSLER.  
COMPOUND FIRE KINDLER.  
APPLICATION FILED JAN. 15, 1915.

1,189,089.

Patented June 27, 1916.

*Fig. 1.*



*Fig. 2.*



*Fig. 3.*



Witnesses

Paul W. Hayd  
J. B. Banning

Inventor  
C. F. Geissler.

By *A. Knudsen, Jr.*  
Attorney

# UNITED STATES PATENT OFFICE.

CHRISTOPHER F. GEISSLER, OF ST. LOUIS, MISSOURI.

## COMPOUND FIRE-KINDLER.

1,189,089.

Specification of Letters Patent. Patented June 27, 1916.

Application filed January 15, 1915. Serial No. 2,397.

To all whom it may concern:

Be it known that I, CHRISTOPHER F. GEISSLER, a citizen of the United States, residing at St. Louis, State of Missouri, have 5 invented certain new and useful Improvements in Compound Fire-Kindlers; and I do hereby declare the following to be a full, clear, and exact description of the invention, such as will enable others skilled in 10 the art to which it appertains to make and use the same.

This invention relates to compound fire kindlers, and the principal object of the invention is to provide a fire kindling which 15 can be produced at low cost and which will be reliable and efficient for its purpose.

In carrying out the invention, the ingredients and the relative proportions of the ingredients are as follows:

|                      |            |
|----------------------|------------|
| 20 Dry stable manure | 48 pounds. |
| Resin                | 4 pounds.  |
| Pitch                | 2 pounds.  |
| Crude petroleum oil  | 1/4 pound. |

25 The manner of mixing the ingredients is as follows: The resin, pitch, and crude petroleum oil are heated to a melted condition and are then mixed with the dry stable manure. When thus mixed a semi-plastic condition is attained and the materials are placed in molds which will form the kindlers into briquets of about six ounces each and having indentations or grooves whereby 30 they may be separated for use. For the purpose of molding the compound I make use of a mold, such as is shown in the accompanying drawing.

Figure 1 is a sectional view taken through 40 a mold and cover therefor and showing the fire-kindling compound in the mold, Fig. 2 is a perspective view of the cover for said mold, and Fig. 3 is a perspective view of

one of the blocks or briquets of fire-kindling separated from the others after molding. 45

Referring to the drawing the numeral 1 designates the bottom of the mold, which may be in the form of a box of the required size for forming a number of briquets, said briquets being practically six inches long, 50 one and one-half inches thick, and two inches wide. A cover 2 for said mold is provided with a series of V-shaped projections 3 which are designed to make a groove in the briquets 4 at opposite sides thereof so 55 that they can be readily detached along the line 5 from the other briquets after molding. The cover 2 is provided with an upwardly extending flange 6 at one or both ends.

The proportions of materials referred to 60 herein will make about one gross of briquets, that is to say, a hundred and forty-four cakes with twenty-four briquets in each cake. These briquets will burn freely and can be lighted with a match and will start 65 a fire readily.

The materials out of which the kindler is made is inexpensive, and the cost of manufacture is very slight. The relative proportions of materials may be varied with- 70 in wide limits without departing from the spirit and scope of the invention as defined in the claim.

What is claimed is:—

A fire kindler consisting of a solid mass 75 of thoroughly mixed dry stable manure forty-eight pounds, resin, pitch two pounds and crude petroleum oil one-quarter pound combined in substantially the proportions stated. 80

In testimony whereof I affix my signature in presence of two witnesses.

CHRISTOPHER F. GEISSLER.

Witnesses:

C. WM. KOENIG,

J. HENRY KOENIG.